

## UNITED STATES PATENT OFFICE

2,343,039

## ELECTRICAL RESISTANCE ALLOY

Victor O. Allen, Madison, and Joseph F. Polak,  
Newark, N. J., assignors to Wilbur B. Driver  
Company, Newark, N. J., a corporation of New  
Jersey

No Drawing. Application July 9, 1942,  
Serial No. 450,278.

4 Claims. (Cl. 75—171)

This invention relates to electrical resistance alloys and has for its object the provision of a high resistance alloy having a relatively low temperature coefficient of resistivity, particularly in the range of temperatures below about 300° C.

Another object is to provide an electrical resistance alloy suitable for use as a resistor element in electrical devices, apparatus and circuits.

Still another object is to provide an electrical resistance alloy consisting predominately of nickel and containing chromium 10% to 30% in which the normal electrical resistance is materially increased and the temperature coefficient of resistivity is materially lowered without material loss of hot and cold workability.

Other objects and advantages will be apparent as the invention is more fully hereinafter disclosed.

In accordance with these objects, we have discovered that copper and beryllium, in combination, are particularly effective, in alloys of nickel and chromium, as agents for increasing the electrical resistance of the alloy and for lowering the temperature coefficient of resistivity and that, in general, copper in amounts up to 3% and Be in total amounts up to 5%, but Cu and Be combined in total amount not over about 6% may be employed for this purpose without seriously impairing the normal hot and cold workability of the base nickel-chromium alloy.

As one specific embodiment of the present invention, but not as a limitation thereof, the adaptation of the same to a well known nickel-chromium alloy containing 80% Ni and 20% Cr heretofore employed as an electric resistance alloy will be described.

The normal temperature coefficient of resistivity of a nickel-chromium alloy containing 80% Ni and 20% Cr within the temperature range 20°-100° C. is .00014 ohm per ohm per degree centigrade, and the electrical resistance at 20° C. approximates 650 ohms per circular mil foot (C. M. F.). The temperature coefficient of resistivity of this alloy is too high for use as a resistor element in high accuracy electrical devices, apparatus and circuits. It is desired by the practice of the present invention to lower the temperature coefficient of resistivity of this alloy to a value below .00014 ohm. We have discovered that copper and beryllium additions to this alloy in total amount not over about 6% with copper not over about 3% and Be not over about 5%, will effectively lower the temperature coefficient of resistivity of the nickel-

chromium alloy from the normal value of .00014 ohm to a value as low as .00002, and will at the same time markedly increase the electrical resistance of the alloy at any temperature within the range 20° C.-300° C.

In general, the copper and beryllium additions to the alloy are made at the expense of the nickel content of the alloy and may be added in various percentages within the ranges above given and in different relative proportions to obtain a plurality of high resistance alloys of progressively lower temperature coefficients of resistivity and different electrical resistances.

A copper content much in excess of about 3% is undesirable for the reason that the hot workability of the alloy is detrimentally effected. A Be content of much over 5% is undesirable for the reason that both the hot and cold workability of the alloy is detrimentally effected. A

total amount of over about 6% of the two constituents (Be and Cu) is undesirable for the reason that cold drawing properties of the alloy, especially at small diameters, appears detrimentally effected.

As one specific embodiment of the present invention but not as a limitation thereof, as alloy containing 20% Cr, 2% Cu, .50% Be, balance Ni, in wire form, has an electrical resistance of about 670 ohms per circular mil foot at 20° C. and has a temperature coefficient of resistivity of about  $97 \times 10^{-6}$  (.000097).

The austenitic structure and non-magnetic properties of this alloy together with its relatively high electrical resistance and low temperature coefficient of electrical resistance, adapts the alloy for extensive utility as instrument and radio resistors, shunts and similar devices.

We have found that larger amounts of Be in the alloy lower the electrical resistivity to a further extent and that Be about 4% with Cu about 2% gives the highest electrical resistance with the lowest temperature coefficient of resistivity.

Due to the high cost of beryllium and the difficulty of producing and working the high Be content alloy, it is preferred to maintain a Be content of below 1% and a copper content of 1.5 to 2.5% as this relative proportioning of the elements Be and Cu in the Cr.Ni base (Cr 10-30%) appears to provide the best combination of the properties of electrical resistance and temperature coefficient of resistivity at the lowest cost.

In the manufacture of the Cr.Ni alloy containing Be and Cu of the present invention, the Be and Cu, preferably in the form of a beryllium-

copper alloy, is added to the molten CrNi alloy after the molten CrNi alloy has been thoroughly deoxidized and degasified by the usual deoxidizing and degasifying agents heretofore employed for this purpose and insofar as the term "balance Ni" is concerned as it may hereinafter appear in the claims, this term is to be construed as including small fractional percentages of one or more of the elements of the group consisting of Mn, Si, Ti, Zr and B.

Whereas in the above specific embodiment an alloy containing Cr 20% is disclosed, it is believed apparent that the Cr may be varied within the range 10 to 30% with resultant increase and decrease in the Ni balance of the alloy, without essential departure from the present invention, obtaining thereby a variation in the electrical resistance and the specific temperature coefficient of resistivity of the alloy, the effect of the Be and Cu additions on any given CrNi base alloy being substantially the same and equivalent to that indicated for the 80 Ni-20 Cr base alloy of the specific embodiment given, but of a different order.

It is believed apparent, from the above description of the present invention, that the same may be widely varied without essential departure therefrom and all such are contemplated as may fall within the scope of the following claims:—

What we claim is:

1. An electrical resistance alloy characterized by having a temperature coefficient of resistivity below .00014 consisting of chromium 10 to 30%, Be from small fractional percentages up to about 5%, Cu from small fractional percentages up to about 3%, with the total Be and Cu not over about 6%, balance Ni.
2. An electrical resistance alloy characterized by having a temperature coefficient of resistivity below .00014 consisting of chromium about 20%, Be from small fractional percentages up to about 5%, Cu from small fractional percentages up to about 3%, with the total Be and Cu not over about 6%, balance Ni.
3. An electrical resistance alloy characterized by having a temperature coefficient of resistivity below .00014 consisting of Cr 20%, Be from small fractional percentages to 1%, Cu 1.5 to 2.5%, balance Ni.
4. An electrical resistance alloy characterized by having a temperature coefficient of about .000097 consisting of Cr 20%, Be .50% Cu 2%, balance Ni.

25

VICTOR O. ALLEN.  
JOSEPH F. POLAK.